

April 20, 1948.

L. C. WERNER ET AL

2,439,916

METHOD OF SEALING COAXIAL STRUCTURES

Filed March 1, 1945

Fig. 1.



Fig. 2.



Fig. 3.



Fig. 4.



Fig. 5.



BY

*J.W. Neuhause*  
INVENTORS  
L. C. WERNER  
W. S. LUND

ATTORNEY

## UNITED STATES PATENT OFFICE

2,439,916

METHOD OF SEALING COAXIAL  
STRUCTURES

Leo C. Werner and Willard S. Lund, Bloomfield,  
N. J., assignors to Westinghouse Electric Corporation,  
East Pittsburgh, Pa., a corporation of  
Pennsylvania

Application March 1, 1945, Serial No. 580,386

3 Claims. (Cl. 49-81)

1

This invention relates to a method of sealing coaxial structures and more particularly to application of glass insulating beads at intervals within a length of tubing between the tubing wall and a coaxial rod within the said tubing.

Heretofore insulating beads have been applied in tubing by applying the glass in desired position and then inserting plungers from opposite ends of the tubing to press the glass, while in plastic condition, and thereby squeeze it into adhering contact with the tube wall. Obviously such a method admits of application of only one bead within a length of tube.

An object of the present invention is to enable a plurality of insulating beads to be formed in a tube.

Another object of the invention is to provide a coaxial structure with an integral length thereof having firmly secured successive insulating beads therein.

A further object of the invention is to provide an improved method for fabrication of coaxial lines with successive beads.

Still further objects of the invention will appear to those skilled in the art to which it appertains as the description progresses both by direct recitation thereof and by implication from the context.

Referring to the accompanying drawing in which like numerals of reference indicate similar parts throughout the several views:

Figures 1 is an elevation of a length of coaxial line broken away at a middle part to show interior structure and fabricated in accordance with our invention;

Figures 2 and 3 are sectional elevations showing the steps of forming the glass buttons on the rod section of the coaxial structure; and

Figures 4 and 5 show successive steps in completion of the seals after insertion of the rod section into the tubular section.

In the specific embodiment of the invention illustrated in said drawing, the reference numeral 10 designates the inner or rod member of a coaxial structure, and numeral 11 denotes the outer or tubular member. The completed structure shows these sections coaxially secured by a plurality of successive glass beads 12 sealed to both members. Heretofore, since it was necessary to insert plungers at opposite sides of the glass bead to force it into sealing contact with the tubular member, only one bead could be applied in a tube and the tubular member therefore had to be undesirably short in order that the inner conductor or member would be adequately sup-

ported to assure its coaxial position. According to the present invention, the inner member or rod is supported by a plurality of meltable beads 12 in a length of outer member, and the length depends only on the capacity of the machine used in its manufacture to receive it. For brevity, said beads will be considered as made of glass, but other materials may be employed having the characteristic of softening under influence of heat to a viscous flowing condition.

Following the successive steps of manufacture, the rod or inner member 10 is first prepared with glass or other buttons thereon, which ultimately become the sealed beads 12. For illustrating completely one exemplification of the method throughout its several steps, Figure 2 indicates that first a cut length of glass tubing 12a is applied to the rod 10 at the position where a bead is desired. By flame 13 or other suitable means, the glass tubing 12a is softened until it wets or adheres to the rod with the rod rotating as indicated by arrow 200 in Fig. 2. Successive lengths of glass tubing 12a are similarly applied along the rod at all places where beads are desired. Each length of glass tubing 12a thus applied to the rod is then built up between its ends by addition of more glass from a stick 14 by use of flame 15 or other suitable means until a button 12b of desired bulk and diameter is formed. Preferably the addition of glass from stick 14 is accomplished while rod 10 is rotating, as indicated by arrow 210, so the forming operation will result in a circular and coaxial button 12b, the diameter of which is limited to less than, but substantially equal to the inside diameter of the tubular member 11 into which the rod, with its several buttons formed thereon, is next inserted.

Both the rod or inner member 10 and the tube or outer member 11 are preferably secured by suitable means, of which chuck 16 is indicative, to the rotating head stock of the machine so that both will be positively rotated and at the same number of revolutions per minute. The tube or outer member 11 is pressed longitudinally toward the chuck by a rotatable tail stock spindle 18. An electrical coil 17 for high frequency induction heating is applied around the tube, loose with respect thereto so as not to interfere with rotation of the tube while the coil remains fixed. With the apparatus thus arranged, the coaxial members are thereupon, as indicated by arrow 220 in Fig. 4, rotated simultaneously at a slow speed and heating is applied as by the electrical high frequency induction from coil 17. The glass buttons 12b becomes hot from this heating,

and at the stage when the glass begins to soften and become soft, the apparatus is speeded up to high speed, say about 2,000 revolutions per minute. The rotation at this increased speed is indicated by arrow 230 in Fig. 5. By virtue of this increased speed, the softness of the glass and centrifugal action, the glass flows into forceful and wetting engagement with the interior surface of the tubular member 10 and seals therewith as final beads 12 above mentioned. When the seal is effected, the rotation and heat are discontinued.

It will be observed that the glass buttons 12<sup>b</sup>, by having substantially the inside diameter of the tube 10, maintain the rod coaxial to the tube, and that this coaxial relationship is maintained as the glass softens during rotation and heating while effecting the seal. Thus the final assembly provides a coaxial structure with a plurality of successive beads maintaining the coaxial relationship of tube and rod. The heating, rotation and centrifugal action during the sealing operation are equally effective upon all the buttons, and therefore the several beads formed are all equally sealed and have corresponding configurations and afford equal spacing and support for the rod within the tube.

We claim:

1. A method of sealing coaxial structures having inner and outer members comprising applying a plurality of meltable buttons on the inner member of said structure, inserting the inner member into the outer member, rotating said members while heating the meltable buttons to a viscous flowing temperature, and engaging the buttons in flowing condition centrifugally against the outer member of the coaxial structure.

2. A method of sealing coaxial structures having inner and outer members, comprising applying a plurality of meltable buttons on the inner member of said structure, inserting the

inner member into the outer member, rotating said members and simultaneously heating the meltable buttons to a viscous flowing temperature, engaging the buttons in flowing condition centrifugally against the inner wall of the outer member of the coaxial structure, and continuing application of heat and centrifugal action on the buttons until they wet and seal to said inner wall and form beads sealed thereto.

3. A method of sealing coaxial structures having inner and outer members, comprising first sealing lengths of glass tubing to the inner member at successive intervals where beading is desired, building up the diameter of glass as a button on each length of tubing, inserting the inner member with the built-up buttons thereon into the outer member, rotating said members, and heating said buttons and centrifugally flowing the glass thereof into sealing engagement with the outer member.

LEO C. WERNER.  
WILLARD S. LUND.

#### REFERENCES CITED

25 The following references are of record in the file of this patent:

#### UNITED STATES PATENTS

|    | Number    | Name               | Date          |
|----|-----------|--------------------|---------------|
| 30 | 1,271,245 | Recklinghausen     | July 2, 1918  |
|    | 1,639,575 | Robinson           | Aug. 16, 1927 |
|    | 1,844,936 | Hotchkiss          | Feb. 16, 1932 |
|    | 2,048,556 | McArthur           | July 21, 1936 |
|    | 2,138,224 | Barasch            | Nov. 29, 1938 |
| 35 | 2,202,337 | Cohn               | May 28, 1940  |
|    | 2,276,218 | Lemmens            | Mar. 10, 1942 |
|    | 2,394,398 | Mouromtseff et al. | Feb. 5, 1946  |

#### FOREIGN PATENTS

|    | Number  | Country       | Date          |
|----|---------|---------------|---------------|
| 40 | 198,322 | Great Britain | July 26, 1923 |
|    | 455,101 | Great Britain | Oct. 14, 1936 |